

Sept. 4, 1956

T. A. MATTHEWS II

2,761,765

**I. A. MATTHEWS II** 2,7  
COMPOSITION AND METHOD OF INHIBITING THE CORROSION  
OF FERROUS EQUIPMENT USED IN THE REGENERATION AND  
BOILING OF ALKALI METAL SOLUTIONS

Filed Oct. 28, 1952

4 Sheets-Sheet 1



**FLANGE IRON**  
**FIG. 1**

*INVENTOR.*

BY THOMAS A. MATTHEWS II

Edward H. Bay

**ATTORNEY**

Sept. 4, 1956

T. A. MATTHEWS II

2,761,765

I. A. MATTHEWS II 2,7  
COMPOSITION AND METHOD OF INHIBITING THE CORROSION  
OF FERROUS EQUIPMENT USED IN THE REGENERATION AND  
BOILING OF ALKALI METAL SOLUTIONS

Filed Oct. 28, 1952

4 Sheets-Sheet 2



S.S. 304  
FIG. 2

*INVENTOR.*

BY THOMAS A. MATTHEWS II

Edward F. Lang

**ATTORNEY**

Sept. 4, 1956

T. A. MATTHEWS II

2,761,765

COMPOSITION AND METHOD OF INHIBITING THE CORROSION  
OF FERROUS EQUIPMENT USED IN THE REGENERATION AND  
BOILING OF ALKALI METAL SOLUTIONS

Filed Oct. 28, 1952

4 Sheets-Sheet 3



CARPENTER 20  
FIG. 3

INVENTOR.

BY THOMAS A. MATTHEWS II

Edward H. Lang

ATTORNEY

Sept. 4, 1956

T. A. MATTHEWS II

2,761,765

COMPOSITION AND METHOD OF INHIBITING THE CORROSION  
OF FERROUS EQUIPMENT USED IN THE REGENERATION AND  
BOILING OF ALKALI METAL SOLUTIONS

Filed Oct. 28, 1952

4 Sheets-Sheet 4



AVERAGE OF MONEL, INCONEL & NICKEL  
FIG. 4

INVENTOR.

BY THOMAS A. MATTHEWS II

*Edward H. Lang*  
ATTORNEY

1

2,761,765

**COMPOSITION AND METHOD OF INHIBITING THE CORROSION OF FERROUS EQUIPMENT USED IN THE REGENERATION AND BOILING OF ALKALI METAL SOLUTIONS**

Thomas A. Matthews II, Crystal Lake, Ill., assignor to The Pure Oil Company, Chicago, Ill., a corporation of Ohio

Application October 28, 1952, Serial No. 317,277

8 Claims. (Cl. 23—184)

This invention relates to a method and a novel inhibitor for reducing the corrosion of ferrous metal equipment used in the processing and handling of solutions containing active percentages of caustic alkali. Specifically the invention comprises a method of inhibiting the corrosion of ferrous equipment used in the regeneration and boiling of alkali solutions containing large and active amounts of alkali, which alkali solutions may or may not contain solubility promoters and oxidation catalysts for the sweetening of hydrocarbon oils or ingredients added to facilitate the removal of sulfur compounds from hydrocarbon oils and gasoline.

Strong alkali solutions, particularly aqueous or alcoholic sodium and potassium hydroxide solutions having 5 per cent or more by weight of active alkali present are known to be corrosive to metal parts, especially ferrous metal parts of equipment used to handle the alkali solutions. The extent of corrosive action of the alkali depends upon its concentration, the temperature and pressure of the system, and the rate of flow or impinging action of the solution on the metal surfaces involved. In the treatment of hydrocarbon oils and distillates for the purpose of removing sulfur compounds or transforming obnoxious sulfur compounds into non-odorous form, it is necessary to regenerate the alkali solutions. This regeneration is accomplished by heating, steam stripping, or air blowing conducted at temperatures above 60° F. and as high as or higher than the boiling point of the alkali solution. During such treatment, the alkali solution is generally circulated through a packed tower or through a bubble tower, and portions thereof recycled to insure adequate regeneration. This necessitates the use of piping and pumps to convey the heated alkali solutions. Severe corrosion of the pumping equipment and metal conduits has been experienced in such operations. The used alkali solutions from such operations contain various sulfur compounds including mercaptans, mercaptides, and disulfides which tend to increase the corrosiveness of the solutions. In addition, certain amounts of dissolved oxygen, various solubility promoters, oxidation catalysts, along with bits of extraneous matter, may be present which increase the corrosiveness and add to the difficulties attendant to attaining a regenerated alkali which is clear and clean, free of sedimentary materials, and readily reused. The boiling and steam stripping to which these alkali solutions are subjected during regeneration presents an atmosphere which is especially corrosive to ferrous metal surfaces and results in many instances in the formation of precipitates which render it colored and often containing sediments making it unfit for contacting hydrocarbons.

To increase the life of the pumps, conduits, and other handling equipment subjected to the above conditions, it has been the practice to fabricate these pieces of equipment from corrosion-resistant stainless steel alloys at considerable expense. Even certain stainless steel alloys are attacked by hot caustic under extreme conditions and often the use of a noble metal alloy promotes the severe

2

corrosion of adjacent parts made of base metals. During the course of investigating the rate of corrosion of ferrous metals in contact with boiling strong caustic alkali solutions, the observation was made that the rate of corrosion increases rapidly during the first few hours of contact and then levels off at a much reduced rate with the passage of time. A study of this phenomenon was made by applicant in order to find an inexpensive means for overcoming the corrosion problem.

10 One explanation for the decreased rate of corrosion over extended periods of time is the formation of a protective film over the metal surface which stops or slows up further attack by the alkali. In an effort to find conditions which demonstrate the true rate of corrosion of these ferrous metals in order to study the actual effectiveness of experimental oxidation and corrosion inhibitors, experiments were conducted using an abrasive in the form of ferric oxide in the alkali solutions under test on the theory that the abrasive would remove the partially protective metal film that seemed to be forming. It was found that, contrary to these expectations, the iron oxide acted in an opposite manner and produced a marked reduction in the corrosion rate. The degree of reduction in corrosion rate was further found to be a maximum with certain optimum concentrations of the iron oxide present in the alkali solution.

Accordingly, it is a fundamental object of the present invention to provide a method of preventing the corrosion which takes place in the boiling of active alkali solutions.

15 A second object of the invention is to provide a method of preventing corrosion of equipment used in the regeneration of alkali sweetening solutions or alkali desulfurizing solutions which have been used in the treatment of hydrocarbons.

20 A further object of the invention is to provide a method of inhibiting the corrosion occurring during the regeneration of alkali solutions and maintaining the solutions in clear, clean, usable condition.

25 Another object is to provide a composition for use in mitigating corrosion of ferrous metal surfaces by alkali solutions.

30 Other objects and advantages of the invention will appear in part or be obvious from the following description.

35 The invention, accordingly, comprises the discovery that the corrosive action of alkali solutions on ferrous metal surfaces may be mitigated by the presence of small but sufficient amounts of red iron oxide ( $Fe_2O_3$ ) and/or 40 the so-called alkali metal ferrites, sodium, potassium, and lithium ferrites, which may be designated by the formula  $Na_2Fe_2O_4$ . The invention has as its embodiments, the process for inhibiting the corrosion of ferrous equipment used in handling alkali solutions, including such processes 45 as the regeneration of alkali used in treating hydrocarbon oils; and the product therefor comprising a composition characterized by its utility in mitigating this type of corrosion.

50 The process includes the several steps to be described and the relation of one or more of such steps to each of the others thereof, which will be exemplified in the method hereinafter described and defined in the claims.

In the drawings,

55 Figure 1 is a graph of weight loss of flange iron samples in contact with hot caustic solution plotted as ordinates against the time in hours plotted as abscissas.

Figure 2 is a graph of weight loss vs. time in hours as determined for stainless steel 304.

Figure 3 is a graph of weight loss vs. time in hours as determined for Carpenter 20, a stainless steel alloy.

Figure 4 represents a graph of the average weight losses

of a number of nickel samples in contact with hot caustic solution plotted as ordinates against the time in hours plotted as abscissas.

Typical examples of industrial processes wherein hot alkali solutions may cause corrosion problems as aforementioned and which may be overcome by the practice of the present invention are those processes employing caustic scrubbing to remove hydrogen sulfide and the majority of the more soluble sulfur compounds and such processes as the Solutizer process, the Unisol process, and the Mercapsol process. The alkali solutions used in these processes may comprise a plain solution of sodium or potassium hydroxide or may also contain various amounts of alcohols, solubilizers, and oxidation catalysts. Although the present invention is intended to embody the prevention of corrosion of ferrous equipment during contact with hot active alkali solutions from whatever source, it will be demonstrated by reference to alkali solutions which are used in the Mercapsol process. The type of solution used in the alkali sweetening of hydrocarbons includes generally an aqueous solvent which may or may not contain an alcohol, having 5 to 50 per cent of caustic alkali usually in the form of sodium hydroxide and depending upon the type of treating process contemplated, up to about 3 per cent of organic catalytic agents, such as hydroquinone, naphthoquinone, wood tars, catechol, aromatic quinone-forming compounds, anthraquinone, and derivatives of these quinones and quinone-forming compounds which have been found useful as accelerators. Such alkali solutions may also contain thiophenolic compounds, thiocresols, alkali metal soaps of naphthenic acids and of unsaturated organic acids, reaction products of alkali and natural or synthetic shellac, copal, acidic petroleum oxidation products, alkali metal salts of high boiling tar acids, rosin, yacca gum, acid oils, and alkali metal phenolates. The solution may also contain other ingredients which have the effect of improving the efficiency of the extraction. Typical of the processes employing this type of solution in hydrocarbon treatment and also including operations for the regeneration of used alkali solutions therefrom are those described in United States Patents 2,292,636 of August 11, 1942, to Lawrence M. Henderson and George W. Ayers, Jr.; 2,297,621 of September 29, 1942, to Lawrence M. Henderson and George W. Ayers, Jr.; and 2,314,919 of March 30, 1943, to Donald C. Bond, George W. Ayers, Jr., and Lawrence M. Henderson.

It is known in the prior art to use many different inorganic salts as inhibitors against various corrosive atmospheres in various systems. United States Patent 2,297,666 of September 29, 1942, to Aaron Wachter, employs sodium nitrite in oil pipe lines. United States Patent 2,153,952 of April 11, 1939, to Alfred L. Bayes, employs sodium nitrate in anti-freeze solutions and Patent 2,135,160 dated November 1, 1938, to Herman Beekhuis, discloses sodium dichromate to inhibit the corrosiveness of ammonium nitrate systems. The use of red iron oxide as a paint pigment is well established and numerous metal protective pigments comprising metal oxides have been used as constituents of primary coats applied to metallic surfaces for the purpose of inhibiting or passivating various kinds of corrosive atmospheres. Lead and zinc pigments, for example, are known for their inhibitive nature. Iron oxides are generally known as neutral pigments. However, it has been observed that strong caustic solutions will actually remove red iron oxide paint and many other protective coatings from metal surfaces.

The state of the art previously outlined emphasizes the fact that the problem of the inhibition of corrosion is one of empirical phenomenon and each particular situation or environment creates its own peculiar corrosion problem requiring specific and exacting solutions. Each problem of the inhibition of corrosion in a given environment, therefore, calls for a process which is designed specifically to meet that problem. A given corrosion

inhibitor may be very useful in a certain application but oftentimes if that inhibitor is employed in what would appear to be an analogous situation or atmosphere the usefulness disappears. In United States Patent 2,556,387 of June 12, 1951, to George W. Ayers, Erskine E. Harton, and Louis R. Mazurk, it is pointed out that sodium phosphate and sodium chromate, which are very well known inorganic salt corrosion inhibitors, were found to be worse than useless in preventing the corrosion of ferrous equipment used in the regeneration and boiling of alkali metal solutions. That patent is directed to the use of alkali metal nitrites to reduce the corrosion of boiling caustic alkali solutions on the ferrous vessels.

The present invention and its applicability to the inhibition of corrosion of ferrous materials by caustic solutions containing various extraneous materials is best understood and demonstrated by reference to the following examples and tables.

A five-gallon stainless steel pail thoroughly insulated with magnesia and fitted with a stainless steel cover and having a tight fitting Tygon tubing gasket was equipped with 1000 watt heaters, a mercury thermoregulator with an electronic relay, stainless steel sample racks, and a water coil. The apparatus was designed to study the rate of corrosion under conditions of no agitation, mild agitation, and extreme agitation. For the latter purpose, the apparatus was equipped with a  $\frac{1}{4}$  H. P. motor driving a rotating shaft through an idler pulley, which shaft suspended a disc type turbine in immersion contact with the alkali solution for rotating samples therein. Various samples of ferrous metals and ferrous metal alloys were subjected to contact with a typical corrosive caustic alkali solution, known as Mercapsol solution, maintained at about 230° F. (boiling temperature) for from over 200 hours to as much as 1235 hours contact time.

The Mercapsol solution used in these tests contained 19.3 per cent sodium hydroxide, 10 per cent cresols, 15 per cent naphthenic acids, and 55.7 per cent water. The 40 Baumé gravity was maintained at approximately 25.5° by daily addition of water, which was lost at about 0.3 weight per cent per day. During the runs, the temperature remained between 220° and 230° F. Four removable baffles were used to prevent vortexing during mixing. Teflon plastic washers were used to suspend the samples and insulate the bolted samples from the turbine. The Mercapsol solution had no effect on this plastic after weeks of immersion.

Each sample before testing was first rubbed with steel wool and emery cloth, then pickled in hot hydrochloric acid solution, rinsed with water and acetone, dried, and weighed. After immersion for about 70 hours, the samples were removed, washed with water and acetone, and dried. During this operation they were rubbed briskly with a cloth to remove any reasonably loose scale. Any adherent scale remaining was included in the weight determinations made. The weight of each sample was taken and the samples were immersed for further contact with the alkali. This procedure provided data relating weight loss with time. All samples were given this same treatment regardless of the degree of agitation which was applied during the tests.

The condition of no agitation represents one wherein the samples were hung in a static solution. The condition of mild agitation wherein the samples are hung in a solution surrounding a mixing turbine and convection currents are allowed to mildly agitate the solution. Conditions of more extreme agitation are represented by the amount of travel in lineal feet per second of the samples when fastened to the mixing turbine.

The following table sets forth an analysis of the samples of ferrous materials used in the experiments.

TABLE I

*Chemical analysis of steels and nickel alloys  
(rolled plate)*

| Type of Steel   | C     | Si   | Mn   | S     | P     | Cr    | Ni    | Cb   | Mo   | Cu   | Fe   | W   |
|-----------------|-------|------|------|-------|-------|-------|-------|------|------|------|------|-----|
| Flange iron     | 0.17  |      | 0.42 | 0.03  | 0.012 |       |       |      |      | 99.4 |      |     |
| 410             | 0.07  | 0.35 | 0.45 | 0.005 | 0.012 | 13.16 | 0.26  |      |      | 86.1 |      |     |
| 304             | 0.060 | 0.69 | 0.66 | 0.013 | 0.019 | 18.44 | 9.06  |      |      | 71.1 |      |     |
| Carpenter 20    | 0.07  | 1.0  |      |       |       | 20.0  | 29.0  |      | 2.0  | 3.0  | 45.0 |     |
| 316             | 0.058 | 0.52 | 1.65 | 0.006 | 0.018 | 17.6  | 12.9  |      | 2.27 |      | 65.0 |     |
| 304 ELC         | 0.03  | 0.49 | 1.37 | 0.16  | 0.24  | 18.79 | 9.15  |      |      |      | 69.8 |     |
| 310             | 0.127 | 1.0  | 1.97 | 0.10  | 0.30  | 24.07 | 21.63 |      |      |      | 50.8 |     |
| 316 ELC         | 0.03  | 0.66 | 1.99 | 0.013 | 0.024 | 17.49 | 13.79 |      | 2.5  |      | 63.5 |     |
| 347             | 0.04  | 0.70 | 1.61 | 0.01  | 0.025 | 18.35 | 10.96 | 0.86 |      |      | 67.4 |     |
| Worthite        | 0.07  | 3.3  | 0.6  |       |       | 20.0  | 24.0  |      | 3.0  | 1.7  | 47.0 |     |
| Illium-G        |       | 1.0  | 1.0  |       |       | 21.0  | 60.0  |      | 6.0  | 4.0  | 6.0  | 1.0 |
| Nickel-Wrought  | 0.05  | 0.05 | 0.25 |       |       |       | 99.4  |      |      | 0.1  | 0.15 |     |
| Monel-Rolled    | 0.15  | 0.1  | 1.0  |       |       |       | 67.0  |      |      | 30.0 | 1.4  |     |
| Inconel-Wrought | 0.08  | 0.25 | 0.25 |       |       | 14.0  | 78.0  |      |      | 0.2  | 7.0  |     |

Some of the metal samples selected, as, for example, Carpenter 20 and alloy steel 304 and 316, where chosen for their extreme resistance to this type of caustic corrosion and a comparison is made to show the relative effectiveness of the corrosion inhibitor of the present invention in bringing flange iron, a typical ferrous metal alloy which is readily corroded, to corrosion resistance comparable to that of the more resistant and more expensive alloy steels. The results of these experiments are set forth in the following table.

of ferrous metal alloys in contact with Mercapsol solution at 230° F. with varying degrees of agitation, it is seen that the total immersion of stainless steels 410, 316, 316 ELC, 304, 304 ELC, 347, 310, and Carpenter 20 under static conditions gave erratic results. Under these conditions, all the steels gave low values of corrosion after a black, adherent protective film had formed. The rate of corrosion as represented in inches per year varied from 0 to 0.00069 for these metals with the protective film and the initial rate of corrosion before film formation was

TABLE II  
*Rate of corrosion of ferrous metals in IPY  $\times 10^4$*

| Run No.        | Before Film Formation |                |               | After Film Formation |                |               | 7     | 8     | 9                                   | 10                                   | 11                                   | 12   | 13  | 14   | High-Speed Runs--11 Feet per Second |                                      |                                      |                                      |
|----------------|-----------------------|----------------|---------------|----------------------|----------------|---------------|-------|-------|-------------------------------------|--------------------------------------|--------------------------------------|------|-----|------|-------------------------------------|--------------------------------------|--------------------------------------|--------------------------------------|
|                | 1                     | 2              | 3             | 4                    | 5              | 6             |       |       |                                     |                                      |                                      |      |     |      | 1.0 Wt. Percent RSH                 | 0.18% Fe <sub>2</sub> O <sub>3</sub> | 0.18% Fe <sub>2</sub> O <sub>3</sub> | 0.18% Fe <sub>2</sub> O <sub>3</sub> |
| Run No.        |                       |                |               |                      |                |               |       |       |                                     |                                      |                                      |      |     |      |                                     |                                      |                                      |                                      |
| Time, Hrs.     | 75                    | 75             | 75            | 355                  | 355            | 355           | 394   | 288   | 262                                 | 256                                  | 1,235                                | 428  | 501 | 275  |                                     |                                      |                                      |                                      |
| Type of Steel  | No Agitation          | Mild Agitation | 2.54 ft. sec. | No Agitation         | Mild Agitation | 2.54 ft. sec. | Blank | Blank | 0.6% Fe <sub>2</sub> O <sub>3</sub> | 0.21% Fe <sub>2</sub> O <sub>3</sub> | 0.04% Fe <sub>2</sub> O <sub>3</sub> |      |     |      | 1.0 Wt. Percent RSH                 | 0.18% Fe <sub>2</sub> O <sub>3</sub> | 0.18% Fe <sub>2</sub> O <sub>3</sub> | 0.18% Fe <sub>2</sub> O <sub>3</sub> |
| Flange Iron #1 | 36.0                  | 60.0           |               | 3.5                  | 2.8            |               | 84.7  | 89.2  | 7.2                                 | 5.2                                  | 16.8                                 | 5.8  | 4.2 | 0.0  |                                     |                                      |                                      |                                      |
| Flange Iron #2 |                       |                |               |                      |                |               |       |       |                                     |                                      | 18.0                                 | 6.1  | 4.6 | 0.0  |                                     |                                      |                                      |                                      |
| 410            | 4.5                   | 21.0           | 90.0          | 2.8                  | 1.2            | 4.1           | 64.6  | 63.9  | 4.3                                 | 46.4                                 | 21.1                                 | 17.3 | 8.1 | 2.7  |                                     |                                      |                                      |                                      |
| 304            | 33.0                  | 87.0           | 131.0         | 0.036                | 1.1            | 3.1           | 6.3   | 5.6   | 1.6                                 | 3.5                                  | 3.1                                  | 10.3 | 0.8 | 1.3  |                                     |                                      |                                      |                                      |
| Carpenter 20   | Nil                   | 16.0           | 51.0          | 0.27                 | 0.036          | 0.0           | 2.1   | 1.6   | 2.4                                 | 3.4                                  | 2.0                                  | 37.5 | 4.3 | 17.0 |                                     |                                      |                                      |                                      |
| Avg. Nickel    |                       |                |               |                      |                |               | 0.07  | 0.04  | 1.1                                 | 1.4                                  | 0.5                                  | 0.0  | 6.0 | 1.6  |                                     |                                      |                                      |                                      |
| 316            | 22.0                  | 68.0           | 178.0         | 0.036                | 1.3            | 4.0           |       |       |                                     |                                      |                                      |      |     |      |                                     |                                      |                                      |                                      |
| 304 ELC        | 45.0                  | 87.0           | 110.0         | 1.3                  | 1.2            | 2.2           |       |       |                                     |                                      |                                      |      |     |      |                                     |                                      |                                      |                                      |
| 310            | 2.8                   | 40.0           | 98.0          | Nil                  | 1.7            | 6.4           |       |       |                                     |                                      |                                      |      |     |      |                                     |                                      |                                      |                                      |
| 316 ELC        | 18.0                  | 69.0           | 158.0         | 0.33                 | 1.7            | 6.9           |       |       |                                     |                                      |                                      |      |     |      |                                     |                                      |                                      |                                      |
| 347            | 29.0                  | 89.0           | 142.9         | 1.1                  | 1.8            | 4.70          |       |       |                                     |                                      |                                      |      |     |      |                                     |                                      |                                      |                                      |
| Worthite       |                       | 24.0           |               |                      | 0.036          |               |       |       |                                     |                                      |                                      |      |     |      |                                     |                                      |                                      |                                      |
| Illium-G       |                       | 2.2            |               |                      | 0.038          |               |       |       |                                     |                                      |                                      |      |     |      |                                     |                                      |                                      |                                      |

<sup>1</sup> Tert-octyl mercaptan.

<sup>2</sup> Tert-butyl mercaptan.

<sup>3</sup> Tert-hexyl mercaptan (under N<sub>2</sub> atm.).

All determinations were made in an atmosphere of air except run No. 14 wherein an atmosphere of nitrogen was used. During the last 378 hours of run No. 11 with flange iron and all of runs 12, 13, and 14, two flange iron samples were tested, one insulated from the stainless steel disc turbine and designated flange iron #1, and the other not insulated and designated flange iron #2, giving a direct comparison in corrosion rates under otherwise identical conditions. This caused no apparent change in the corrosion rate as evidenced from the sample in the insulated state. In run No. 12, from the 305 hour time to 428 hour time, the following sulfur compounds were found by analysis to be present: 0.6 weight volume per cent of sulfate and 0.1 weight volume per cent of S<sub>2</sub>O<sub>3</sub>. In run No. 13, iron sulfide (FeS) was present from 351 hours to 501 hours in 0.4 weight per cent concentration. A complete fresh charge of Mercapsol solution was added at 334 hours at run No. 11. No make-up inhibitor was added or needed during the determinations.

Referring to Table II, runs 1 through 6, having as their objective the determination of the rate of corrosion

larger (0 to 0.0178 IPY) with the time for film formation being 70 to 300 hours. The samples all lost more weight immediately after immersion in the hot Mercapsol solution than after passivation by the formation of a protective film. The film formed was a black scale, not readily attacked by strong acids and difficult to remove by rubbing with an emery cloth. Illium-G is the only alloy devoid of such film. For these determinations, it can be concluded that the time of passivation and the rate of corrosion after passivation are dependent on the degree of agitation during the tests. Conditions of mild agitation (runs 2 and 5) gave more consistent results, while rotation of the samples at a constant speed of 2.54 feet per second through the Mercapsol (runs 3 and 6) gave the most consistent data. These determinations, although giving accelerated rates of corrosion, were still not equivalent to the rates of corrosion experienced in certain pipe fittings and other equipment made of flange iron in a Mercapsol unit.

Consequently, in a further study of the corrosion problem in which additional determinations were made

to ascertain the effect of ferric oxide alone and the addition of other corrosive sulfur compounds, the unusual inhibiting effect of ferric oxide was discovered. The efficacy of this substance as a corrosion inhibitor is illustrated by runs 8 through 14, inclusive, in Table II. Herein it is seen that the corrosion rates are reduced to about one-twelfth that of the flange iron in straight Mercapsol solution. Although the concentration of ferric oxide was varied from 0.04 to 0.6 weight per cent and the relative corrosivity of the caustic increased by addition of mercaptan, no conditions were found which disturbed the inhibiting action of the ferric oxide at optimum concentrations of inhibitor. It is to be observed that with a concentration of ferric oxide of around 0.18 weight per cent, the maximum reduction in corrosion rate 15 amounting to about one-sixteenth that of the blank is obtained.

From these experiments, it is seen that small quantities of inhibitors of the present invention may be used to accomplish the desired result. Since ferric oxide is soluble in alkali solutions with the formation of alkali metal ferrites, the sodium salt being representative,  $\text{Na}_2\text{Fe}_2\text{O}_4$ , it is apparent that the inhibiting action may be attributed to either or both of these materials. No added results are obtained by using quantities of ferric oxide in excess of the range of optimum concentrations. The presence of small amounts of suspended particles of ferric oxide in the alkali solution is not deleterious, except that the use of such quantities of ferric oxides or alkali metal ferrites as to form a sludge which may foul the conduits or pumps in the system is to be avoided. The concentration of the ferric oxide either as such or in the form of the alkali metal ferrite may, therefore, be as low as 0.04 weight per cent, and it is immaterial whether quantities are used in excess of the solubility of the ferric oxide in the alkali. For maximum protection under most conditions it is contemplated that from 0.04 to 0.6 weight per cent of ferric oxide, for example, may be used, although the preferred range is about 0.1 to 0.2 weight per cent to obtain the most efficient inhibition.

The optimum concentration of 0.18 weight per cent of inhibitor as used in accordance with this invention serves to bring the rate of corrosion of flange iron down to that of the expensive stainless steels. In addition, the inhibitor of this invention successfully reduces the rate of corrosion of such alloys as that represented by 304 and 410. The conclusions herein drawn are verified by reference to the graphs, Figures 1, 2, 3, and 4.

Electron diffraction analyses were conducted to determine the composition of the scale that was formed on the metal surfaces. These analyses showed that the scale was composed predominantly of ferrosic oxide ( $\text{Fe}_3\text{O}_4$ ) with strong possibilities of some ferrous oxide ( $\text{FeO}$ ). No evidence was found of ferric oxide or sodium ferrites in the scale. This serves to confirm in part the conclusion that the action of the ferric oxide and alkali metal ferrite inhibitors of the present invention is one of true inhibition or negative catalysis and not a mere blanketing of the metal from the influence of the alkali through some type of film formation.

In the graphs, Figures 1, 2, 3, and 4, wherein weight loss in milligrams per square centimeter of sample surface is plotted against time and hours, the various curve numbers shown correspond to the run numbers set forth in Table II. For example, runs No. 7 and 8 of Table II, which are conducted for the various test samples with no inhibitor present, are represented by curves 7 and 8 in each graph for the different alloy samples, and run No. 9, conducted with 0.60 weight per cent of ferric oxide present, is represented by curve 9 in each graph for the indicated alloy, etc. And, likewise, run No. 14, conducted with 0.18 weight per cent of ferric oxide and 1.0 weight per cent of tertiary hexyl mercaptan in an atmosphere of nitrogen, is represented by curve 14. In Figure 1, it will be noted that curves 11, 12, and 13

are shown in duplicate. The left-hand curve of each pair indicates the results of those determinations conducted after removal of the insulating washer from between the sample and the rotating disc turbine. The 5 curves graphically represent the data of Table II and point up the unusual inhibiting effect of ferric oxide in transposing the resistive of flange iron into that approaching the more resistive stainless steel and nickel alloys.

An exemplary operation wherein caustic solutions containing corrosive sulfur compounds are subjected to conditions conducive to the type of corrosion just illustrated by Table II is the regeneration of spent caustic containing about 12 per cent by weight of free alkali and about 0.25 weight per cent of mercaptan sulfur. In such a regeneration system, the spent caustic is withdrawn from storage at a temperature of 60° to 100° F. at a rate of 20 to 30 barrels per hour and is heated to about 220° to 230° F. by indirect heat exchange with steam for entry into an upper section of a regeneration tower operating at about 4 pounds per square inch. Steam at 400° F. is fed to a reboiler operating in connection with the tower to maintain temperatures at about 240° to 245° F. therein. The approximate temperatures at the top and bottom of the tower are maintained at 212° and 250° F., respectively. Hot regenerated, concentrated caustic containing about 0.06 weight per cent of mercaptan sulfur leaves the reboiler, passes in indirect heat exchange with incoming spent caustic, where it drops to a temperature of about 110° F., and passes back to the hydrocarbon 25 treating tower. In such operations, the addition of ferric oxide to the system in accordance with this invention will greatly reduce corrosion.

Regeneration by blowing the spent caustic with an oxygen-containing gas, wherein temperatures of 80° F. 30 and higher are encountered and hot caustic must be circulated by pumps and conduits, comprises another process wherein the present invention may be practiced to reduce corrosion.

The present invention may also be practiced by using 35 separate compositions comprising the inhibitor dissolved or suspended in a suitable vehicle, which compositions may be added to the corrosive alkali metal hydroxide solutions to be inhibited. Suitable vehicles for this purpose may comprise a solvent or suspending medium, as 40 water, oil, aqueous alkali, and portions of the corrosive alkali solution, as the Mercapsol solution. Such solutions of ferric oxide and/or alkali metal ferrites in a vehicle may be prepared in concentrations designed to 45 attain, when added to the corrosive alkali, sufficient inhibitor therein to function in mitigating corrosion.

The rate of corrosion of ferrous metals by alkali solutions increases almost directly with increase in temperature and is most severe at temperatures of 250° F. or higher. However, the invention is not to be limited by 50 any temperature range since caustic solutions exhibit corrosivity at low temperatures, that is, 60° to 100° F., depending on the rate of flow of the caustic through the equipment. In ordinary circulatory systems where caustic solutions are transported from tanks to treating 55 towers and recycling is practiced, the rate of flow of the solutions within the tanks' heating coils, heat exchangers, pumps, and conduits will range from 0 feet per second to 20 to 25 feet per second or higher. The volume rate of feed of caustic solutions through a given system may 60 be as high as 50 to 100 barrels per hour depending on the size of conduit used and the capacity of the system. The degree of turbulence and impingement of caustic against the metal surfaces will vary throughout the system depending on the flow characteristics of the conduits. 65 Since the inhibitors of the present invention are operative under static conditions and shown to be more effective where the degree of turbulence and corrosion are higher, no upper limit need be set on the rate of flow.

The invention is not to be limited by any theories 70 expressed or implied herein. It may be postulated, how-

ever, that several influences or theoretical reactions may be operating singly or in concert to produce the results observed. One contributing cause of the corrosion may be small amounts of oxygen present in the alkali solutions, as evidenced by the reduction in corrosion found in test 14 (Table II) conducted in an atmosphere of nitrogen. Some nickel alloys seem to increase in their rate of corrosion upon the exclusion of oxygen which would suggest the presence of a protective film of nickel oxide as a reactant. The corrosion may be caused by a galvanic action which is upset by the presence of the novel inhibitor of the present invention due to a change in the nature of the scale formation. The influence of hydrogen embrittlement in the presence of sulfides in solution must not be overlooked. The ferric oxide may act to screen the hydrogen ions from the metal or even prevent their formation.

It has been stated that the solution of ferric oxide in alkali produces alkali metal ferrites, and therefore alkali metal ferrites are included as inhibitors herein. Certain alkali metal ferrites decompose in water and are existent in stable form, mainly in strong alkali metal hydroxide solutions, i. e., concentration of alkali of 40 per cent or more. If decomposition of a ferrite solution takes place, there is formed hydrated ferric oxide or ferric hydroxide. Consequently, the invention is not limited to the use of ferric oxide and/or alkali metal ferrites per se, and includes operable concentrations of hydrated ferric oxide which may form from such decomposition and also is directed to those solutions of alkali metal ferrites which are soluble in concentrated alkali without decomposition under the conditions imposing in the system being treated.

What is claimed is:

1. In the method of regenerating spent aqueous alkali solutions which have been used to extract sulfur compounds from hydrocarbon oils without substantial corrosion of ferrous equipment in contact with said solutions, said alkali solutions containing about 5% to about 50% by weight of caustic alkali and containing phenolic organic material, but being substantially free of alkali metal sulfides, the step comprising, incorporating about 0.04 to 0.6% by weight of an inhibiting material of the group consisting of ferric oxide and alkali metal ferrites in said alkali solution throughout said regeneration as a corrosion inhibitor.

2. The method in accordance with claim 1 in which the ferrous metal surface being protected is flange iron

comprising about 99.4% iron, about 0.17% carbon, about 0.42 manganese, and small percentages of sulfur and phosphorus.

5 3. In the method of regenerating spent aqueous alkali solutions used to extract sulfur compounds from hydrocarbon oils wherein said solutions are subjected to heating temperatures ranging from about 212° to 250° F. in contact with ferrous metal surfaces under conditions conducive to corrosion of said surfaces, the improvement comprising maintaining about 0.04 to 0.6 percent by weight of an inhibiting material of the group consisting of ferric oxide and alkali metal ferrite in said alkali solution throughout said regeneration to prevent corrosion of said metal surfaces.

10 4. The method in accordance with claim 3 in which the inhibiting material is ferric oxide in a concentration of about 0.18 percent by weight and said ferrous metal surface is flange iron.

5 5. The method in accordance with claim 3 in which the alkali metal ferrite is sodium ferrite.

6 6. The method in accordance with claim 3 in which the alkali metal ferrite is potassium ferrite.

7 7. The method in accordance with claim 3 in which the alkali metal ferrite is lithium ferrite.

8 8. The method in accordance with claim 3 in which the alkali solution contains about 19.3 percent by weight of sodium hydroxide, 10 percent cresols, 15 percent naphthenic acids, and 55.7 percent water.

#### References Cited in the file of this patent

#### UNITED STATES PATENTS

|           |            |               |
|-----------|------------|---------------|
| 1,883,211 | Wilson     | Oct. 18, 1932 |
| 2,132,585 | Spittle    | Oct. 11, 1938 |
| 2,415,798 | Pye et al. | Feb. 11, 1947 |
| 2,556,387 | Ayers      | June 12, 1951 |

#### OTHER REFERENCES

J. W. Mellor's: "A Comprehensive Treatise on Inorganic and Theoretical Chemistry," vol. 13 (1934), pages 781, 816, 817, 906, Longmans, Green & Co., N. Y.  
 40 "Corrosion Reporter," vol. 1—No. 3, Sept. 1946. Process Industries Quarterly published by International Nickel Co.

Ind. and Eng. Chem. Sept. 1932, pages 1021, 1022.

"Materials of Construction for Chem. Eng. Equipment," published in Chem. and Metallurgical Chem. Sept. 1944, page 125.